# EUROPEAN PATENT SPECIFICATION

(11) **EP 3 026 128 B1**
(45) Date of publication and mention of the grant of the patent: **24.06.2020**
(21) Application number: 14382479.5
(22) Date of filing: 27.11.2014
(51) Int. Cl.: C21D 5/00, C21D 1/20, C21D 1/68, C21D 1/70, C22C 37/04

(54) **A method to control ausferritic as-cast microstructure in ductile iron parts**
Verfahren zur Steuerung einer ausferritischen Mikrostruktur im Gusszustand aus Kugelgrafitteilen
Procédé de commande de microstructure brute ausferritique de pièces en fer ductile

(43) Date of publication of application: 01.06.2016
(73) Proprietor: Fundación Azterlan, 48200 Durango (Bizkaia) (ES); Veigalan Estudio 2010 S.L.U., 48200 Durango (Vizcaya) (ES)
(72) Inventor: Méndez, Susana, 48200 Durango (Vizcaya) (ES); de la Torre, Urko, 48200 Durango (Vizcaya) (ES); Suarez, Ramón, 48200 Durango (Vizcaya) (ES)
(74) Representative: Balder IP Law, S.L.

(56) References cited:
- EP-A1- 2 749 658
- JANOWAK J F ET AL: "APPROACHING AUSTEMPERED DUCTILE IRON PROPERTIES BY CONTROLLED COOLING IN THE FOUNDRY", INTERNATIONAL CONFERENCE ON AUSTEMPERED DUCTILE IRON, XX, XX, 2 April 1984 (1984-04-02), pages 63-69, XP001182603,

## Description

### TECHNICAL FIELD

The present invention relates to the techniques used to obtain ausferritic ductile iron parts, and more particularly to techniques to obtain ausferritic as-cast microstructures without an austempering heat treatment.

### STATE OF THE ART

The possibility to replace some steel applications led to develop a new process to produce a ductile iron with an ausferritic matrix. Its excellent strength/toughness ratio allows eventually replacing casted or forged steel and even aluminum castings by this material, offering to the market components with a higher strength-to-weight ratio and lower price.

For the manufacturing of ausferritic ductile iron with high quality the most common and easiest to reproduce method consists in an austempering process. The ausferritic ductile iron obtained accordingly is usually referred to as austempered ductile iron (ADI). The austempering process is a three step heat treatment which comprises the austenitization of the casting at a temperature higher than 850ºC until the matrix structure attains a reasonably uniform carbon content; quenching to an intermediate temperature range of 260 to 400ºC and tempering, which consists in the transformation to austenitic-ferritic structure at the isothermal temperature. This process increases the final cost of the casting and also the lead time.

Nevertheless, a new process based in the engineered cooling was proposed in EP 2 749 658 A1. The process comprises the following steps:
(i) Casting a melt of a ductile iron alloy in a mould.
(ii) Solidification of the casting in the mould and subsequent cooling until the casting temperature is between 800ºC and 950ºC.
(iii) Shaking out the casting at said temperature between 800ºC and 950ºC.
(iv) Cooling the casting until the temperature of the casting reaches a value between 275ºC to 450ºC with a high enough cooling rate in order to avoid the pearlitic nose.
(v) Introducing the casting in an insulating material and leaving the casting inside for a period of time until a completely ausferritic microstructure is obtained.

By this method ausferritic castings can be produced in as-cast conditions. This engineered cooling reduces the energy required to produce a component (avoiding the austempering heat treatment) and improves the added value of the parts, as well as reducing the lead time. In addition, the entire life-cycle-energy is reduced.

Nevertheless, this process was used for a single alloy and for a specific casting (i.e steering knuckle). However, many automotive castings that are candidates for this technology present geometries with significant thickness variations and consequently with different cooling rates. These differences can complicate or even make impossible the production of fully ausferritic as-cast parts by engineered cooling.

Similar processes are described in JANOWAK J F el al: "Approaching austempered ductile iron properties by controlled cooling in the foundry", Int. Conf. on Austempered Ductile Iron, 2 April 1984, p.63/9 and in U. de la Torre et al: "As-Cast Ausferritic Ductile Iron", Proceedings of the Keith Millis Symposium on Ductile Cast Iron 2013, October 15-17, Nashville, Tennessee.

In sum, a process is needed, which enables to solve in an efficient way, the above mentioned problems of conventional processes for obtaining parts with ausferritic microstructures.

### DESCRIPTION OF THE INVENTION

The present invention provides a method as defined by claim 1. The preferred embodiments are defined in dependent claims 2-11.

### BRIEF DESCRIPTION OF THE DRAWINGS

The drawings comprise the following figures:
Figure 1 shows the cooling curves as a function of the thermal modulus.
Figure 2 shows CCT diagrams for three different alloys.
Figure 3 shows the influence of the alloy content and the thermal modulus on the eutectoid transformation temperature.
Figure 4 shows a graphical description of the calculus of the optimum shakeout temperature.
Figure 5 shows microstructures for different thermal moduli.
Figure 6 shows the evolution of the mechanical properties as a function of the isothermal transformation temperature.

### DESCRIPTION OF A WAY OF CARRYING OUT THE INVENTION

Next embodiments of the invention will be described by way of example, with reference to the above-mentioned drawings showing apparatuses and results according to the invention.

The melts were prepared in a 100 kg medium frequency induction furnace (250 Hz, 100 kW). The metallic charge was made up of low alloyed steel scrap (0.007 % C; 0.002 % Si; 0.17 % Mn; 0.003 % P; 0.006 % S), high purity nickel (99 % min.), FeMo (64.25 % Mo; 2.05 % Si; 0.019 % C; 0.042 % S; 0.030 % P) and copper (99 % min.), in addition to graphite (99 % min; <0.03 % S; <0.04 % H; <0.01 % N) and FeSi75 (74.6 % Si; 0.83 % Al; 0.12 % C). Once the raw materials were melted, the chemical composition was checked and adjusted adding the needed above mentioned materials according to the required carbon, silicon, nickel, copper and molybdenum contents.

The tapping process from the furnace to the ladle was carried out at a temperature range between 1510 and 1530 ºC. The spheroidization treatment was performed following the sandwich methodology, adding 1.2 % (by weight considering the total weight of the treated melt) of a FeSiMg alloy (46.21 % Si, 6.47 % Mg, 0.98 % Ca, 0.67 % Al and 0.97 % RE).

To obtain variable cooling rates, castings presenting different thermal moduli with several geometries were poured. The studied thermal moduli range was between 0.4 cm and 1.5 cm. The produced samples varied from plates (100 x 60 mm²) of different thicknesses to cylinders with different diameters (diameter=height) and keel blocks Y2. The molds were made in all cases of chemically bonded sand.

The inoculation was carried out in mold using 0.2 % (by weight with respect to the total weight of the casting plus feeding and feeling systems) of a Germalloy ingot (71.7 % Si, 3.93 % Al, 0.99 % Ca, Traces % Mg, Traces % RE) or Amerinoc (69.9 % Si; 0.49 % Bi; 0.93 % Al; 1.38 % Ca; 0.24 % Ce; 0.13 % La; 0.19 % Zr; grain size of 0.2-0.5 mm).

The range of chemical compositions in wt% of the cast parts was as follows: 3.58-3.75 % C, 2.00-2.15 % Si, 0.18-0.25 % Mn, 0.007-0.010 % P, 0.006-0.009 % S, 0.038-0.049 % Mg. The alloying elements changed to develop the CCT diagrams were Ni, Cu and Mo and they were on the following ranges: 2.86-5.05 % Ni, 0.01-0.22 % Mo, 0.09-0.90 % Cu.

On the first part of the experiments, in order to develop the CCT diagrams, an early shakeout was applied to all the samples followed by an air cooling. The cooling curve of each casting was recorded by means of a thermocouple (type K) inserted in their thermal centre. With this information, the cooling rate for the different thermal moduli was experimentally calculated on the temperature ranges where the eutectoid transformation takes place. Afterwards, the samples were metallographically analyzed to define if pearlite appeared. This way were defined the pearlitic nose and the minimum cooling rate needed to avoid the formation of this phase as a function of the alloy content. For the metallographic analysis, the specimens were cut and prepared for a visual inspection by means of an optical microscope. The used etchant to reveal the microstructure was Nital 5 %.

The second step of the trials was to define the processing temperatures to obtain an ausferritic microstructure as-cast and relate them to the different thermal moduli of the castings. For that purpose, the alloy that presented a pearlitic nose on more prolonged times was considered, that is (in weight %): 3.63-3.75 % C, 2.04-2.15 % Si, 0.19-0.24 % Mn, 0.007-0.010 % P, 0.006-0.009 % S, 0.042-0.049 % Mg, 2.86-3.01 % Ni, 0.17-0.22 % Mo, 0.09-0.19 % Cu.

The pouring temperature was between 1390 and 1410 ºC. Once poured and solidified, the castings followed a controlled cooling process. At the beginning, all the samples were shaken out at the same instant and air cooled till they reached the temperature range where the ausferrite formation can occur. At this moment, the samples were introduced into an insulating medium presenting a thermal conductivity lower than 0.006 W/mK. The insulating material used for these trials was expanded pearlite with a mesh size less than 5 mm and a density between 40-120 kg/m³. The aim of this step is to maintain a constant temperature to enable the ausferritic reaction to occur. The isothermal transformation time was defined as 90 minutes for all the samples. Finally, after the isothermal process, the samples were air cooled to room temperature. On Figure 1 an example of some cooling curves as a function of the thermal modulus is shown.

With the experimental data, the relation between the shakeout temperature and the thermal modulus was obtained.

Afterwards, taking into account an air cooling after the shakeout process, the isothermal transformation temperature as a function of the thermal modulus was calculated.

Finally, the mechanical properties of the samples were studied. Tensile (10 mm diameter) and hardness specimens were machined from the samples. The ultimate tensile strength (U.T.S.), the yield strength (Y.S.) and the elongation (El.) were measured. In addition, Brinell hardness (HB) measurements were carried out using a 10 mm diameter sphere and a load of 3000 kg.

Regarding the CCT diagrams, the three alloys mentioned on the former sections were considered. The chemical compositions are shown on Table 1.

**Table 1. Chemical composition of the alloys for which the CCT diagrams were developed (wt. %).**

| Alloy | C | Si | Mn | Mg | Ni | Mo | Cu |
|---|---|---|---|---|---|---|---|
| 3.0 % Ni 1.0 % Cu 0.0 % Mo | 3.60-3.73 | 2.00-2.12 | 0.18 - 0.22 | 0.038-0.045 | 2.90-3.05 | <0.02 | 0.94 - 1.01 |
| 5.0 %Ni 1.0 %Cu 0.0 %Mo | 3.58-3.69 | 2.03-2.14 | 0.20 - 0.25 | 0.040-0.049 | 4.95-5.05 | <0.02 | 0.97 - 1.04 |
| 3.0 %Ni 0.0 %Cu 0.2 %Mo | 3.63-3.75 | 2.04-2.15 | 0.19 - 0.24 | 0.042-0.049 | 2.86-3.01 | 0.17 - 0.22 | 0.09 - 0.19 |

On the temperature range between 800 and 500 ºC, cooling rates from 0.2 ºC/s up to 1.3 ºC/s were considered for each alloy. The results are shown on Figure 2.

On the Table 2 the experimental minimum cooling rates for each alloy to avoid the formation of pearlite are shown. In order to simplify the mathematical concepts, the cooling curves on the temperature range between 700 ºC and 600 ºC were considered as straight lines, which is in good accordance with the experimental results. The selected temperature range, takes into account the steps before and during the eutectoid transformation for these alloys.

**Table 2. Minimum cooling rates to avoid the pearlite formation.**

| **Alloy** | **Minimum cooling rate (ºC/s)** |
|---|---|
| 3.0 % Ni; 1.0 % Cu | 1.25 |
| 5.0 % Ni; 1.0 % Cu | 0.60 |
| 3.0 % Ni; 0.2 % Mo | 0.53 |

Considering the studied chemical compositions, an equation to calculate the minimum cooling rate (CRₘᵢₙ) to avoid the pearlitic nose as a function of the nickel, copper and molybdenum contents (Equation 1) was developed.

This equation was validated on the studied composition ranges (3.0-5.0 % Ni; 0.1-1.0 % Cu and 0.0-0.2 % Mo).

On a second step, the thickness window in which this methodology is feasible was defined. The higher the thermal modulus of a casting the longer the solidification process and the lower the cooling rate. The fact that a single casting has different sections and also different thermal moduli, leads to establish a thickness window in which this methodology is feasible.

On the one hand, the shakeout process cannot be carried out at any temperature. The upper limit (1050 ºC) was defined around 50 ºC below the solidus temperature. This is due to the fact that shaking out a casting which is not completely solid can lead to casting defects as microporosity or high thermal stress. The lower limit was defined as 50 ºC over the eutectoid transformation temperature. This temperature is a function of the thermal modulus and the alloy content. The Figure 3 shows the influence of the thermal modulus and the alloy content on the eutectoid transformation temperature.

To define the lower limit of the shakeout temperature, the most restrictive of the curves, which corresponds to the 3.0 % Ni; 0.2 % Cu and 0.0 % Mo alloy, was considered. The following expression was obtained as a function of the thermal modulus (M) (Equation 2). This equation fits the obtained experimental results:

Taking into account the trials carried out using castings with different thermal moduli, the solidification time and the subsequent cooling in the mold till the shakeout temperature was calculated as a function of the thermal modulus. Thermal moduli in the range between 0.4 and 1.5 cm were studied and it was seen that a straight line relation could be defined in order to obtain the shakeout temperature for the different sections of a given casting. This function is shown on the equation 3.

The value of the shakeout temperature for a thermal modulus of 0.6 cm is a constant determined by an iterative calculus method. This reference value is needed to change the moment of the shakeout, which enables to fit, for the different sections, the shakeout temperature into the range defined by the upper and lower limit (when possible).

For a given casting, the model can calculate several shakeout moments that make the process feasible. The iterative method chooses the one that gives the lower shakeout temperature, with the aim of reducing the thermal stress due to a high temperature shakeout.

The result is the shakeout temperature for the minimum and maximum thermal moduli of a casting.

The described calculus regarding the shakeout temperature is shown on Figure 4. It also shows the possibility to change the maximum and minimum thermal modulus of the casting to be considered.

The aim of the cooling process is to obtain fully ausferritic microstructures. Therefore, once defined the alloy to avoid the pearlitic nose and the shakeout temperature as a function of the different thermal moduli of a casting, the next step which has a decisive importance is the isothermal transformation temperature. In this work the temperature at which the different thermal moduli of a casting are to be introduced into an insulating medium was calculated based on the experimental results. On this phase, the model calculates the isothermal transformation temperature as a function of the thermal modulus (Equation 4). ${T}_{isothermal {transformation}_{M}} \left(C\right) = 293.39 ∗ M \left(cm\right) + {T}_{isothermal {transformation}_{0.6 cm}} \left(C\right) - 180$

Following the same methodology as for the shakeout temperature, the value of the isothermal transformation temperature for the modulus 0.6 cm is needed. This reference value fits (when possible) the isothermal transformation temperature of the different moduli into the defined range (explained below).

The isothermal transformation must take place into a determined temperature range to obtain the desired microstructure and thus the mechanical properties that allow meeting the requirements of the ADI materials. In this case the upper limit was considered as 450 ºC, temperature above which it is not considered in the literature that the obtained ausferrite shows the desired mechanical properties. The lower limit is considered as the martensite start formation temperature (M_{S}). For the alloy considered on this part of the work, the Mₛ was defined by means of dilatometry tests in 170 ºC.

Considering the equation No 4 and the limits for the ausferritic reaction, the model defines if the given casting can be produced following this methodology and when feasible, the temperature at which the casting should be introduced into the insulating medium. From the different possibilities that offers the iterative calculus, the optimum solution is the one that enables to obtain the desired mechanical properties in terms of ultimate tensile strength and hardness.

The mechanical properties of the different samples were analyzed by means of tensile and hardness tests. The Table 3 shows the mechanical properties obtained on one of the trials as a function of the thermal moduli of the castings. All the castings were handled together (shaken out and inserted into the insulating medium at the same time).

**Table 3. Mechanical properties as a function of the thermal modulus.**

| **Thermal Modulus (cm)** | **UTS (Mpa)** | **YS (Mpa)** | **E (%)** | **HB** |
|---|---|---|---|---|
| 0.65 | 1020 | 569 | 2.4* | 356 |
| 0.83 | 1040 | 614 | 7.1 | 321 |
| 0.97 | 848 | 548 | 3.9* | 308 |
| 1.07 | 846 | 627 | 7.9 | 288 |
| 1.15 | 822 | 552 | 11.3 | 280 |
| 1.22 | 760 | 552 | 7.9 | 263 |
| 1.28 | 775 | 573 | 7.0 | 266 |

| | | | | |
|---|---|---|---|---|
| *Microshrinkage on the surface of the specimen. | | | | |

It is seen, that depending on the thermal modulus, different ADI grades were obtained. This is due to differences on the processing temperatures of the samples. On the Figure 5 are shown the microstructures obtained for the modulus 0.65 cm and 1.28 cm.

It is observed that the lower the thermal modulus, the greater the lower ausferrite appearance. This results in higher resistance for the lower thermal moduli, but lower toughness. A statistical analysis was carried out with all the data obtained on this work, to relate the process parameters to the mechanical properties. The results of this study are shown on Table 4.

**Table 4. Results of the statistical analysis.**

| | **UTS** | **YS** | **EI** | **HB** | **Thermal Modulus** | **T shakeout** | **T Tempering** | **Nodule count** | **Pear lite** | **Marten site** |
|---|---|---|---|---|---|---|---|---|---|---|
| **UTS** | 1.00 | 0.11 | 0.01 | 0.67 | -0.52 | -0.33 | **-0.59** | -0.30 | -0.59 | -0.22 |
| **YS** | 0.11 | 1.00 | -0.36 | 0.42 | 0.02 | -0.03 | **-0.57** | 0.05 | 0.11 | -0.63 |
| **EI** | 0.01 | -0.36 | 1.00 | -0.45 | -0.07 | -0.04 | **0.60** | -0.44 | -0.03 | -0.29 |
| **HB** | 0.67 | 0.42 | -0.45 | 1.00 | -0.30 | -0.21 | **-0.88** | 0.10 | -0.35 | -0.19 |
| **Thermal Modulus** | -0.52 | 0.03 | -0.07 | -0.30 | 1.00 | 0.89 | 0.45 | 0.52 | 0.38 | - |
| **T shakeout** | -0.33 | -0.03 | -0.04 | -0.21 | 0.89 | 1.00 | 0.46 | 0.39 | 0.23 | -0.42 |
| **T Tempering** | **-0.59** | **-0.57** | **0.60** | **-0.88** | 0.45 | 0.46 | 1.00 | -0.02 | 0.31 | -0.01 |
| **Nodule count** | -0.30 | 0.05 | -0.44 | 0.10 | 0.52 | 0.39 | -0.02 | 1.00 | 0.05 | 0.73 |
| **Pearlite** | -0.59 | 0.11 | -0.03 | -0.35 | 0.38 | 0.23 | 0.31 | 0.05 | 1.00 | -- |
| **Martensite** | -0.22 | -0.63 | -0.29 | -0.19 | -- | -0.42 | -0.01 | 0.73 | -- | 1.00 |

It is seen, that the process parameter that has a greater influence on the mechanical properties is the isothermal transformation or tempering temperature (higher correlation values). For this reason, on the Figure 6, the relationship between the isothermal transformation temperature and the mechanical properties was further analyzed.

The evolution of the elongation is not very clear, presenting a high scattering of the results. This could be due to the high sensitiveness of this property with casting defects like for example microporosity. The yield strength neither presents a clear relationship. It seems to be more or less constant regardless of the tempering temperature. However, the ultimate tensile strength and hardness show a clear tendency linked to the isothermal transformation temperature. The higher this temperature the lower these both properties. This allows assuming that depending on the ADI grade that is being looked for, the optimum transformation temperature will be one or another. Based on the relationship between the isothermal transformation temperature and the thermal modulus, the model will define the optimum isothermal transformation temperature by means of the equation No 4 and the following equations No 5 and 6. $UTS \left(MPA\right) = - 1.2231 ∗ M \left(cm\right) + 1308.2$ $HB = - 0.483 ∗ M \left(cm\right) + 466.34$

All this steps define the different processing parameters in order to obtain fully ausferritic microstructures on all the sections of the casting.

## Claims

1. A method to control the ausferritic as-cast microstructure in a process for obtaining iron parts with sections of different thickness, which comprises:
a) Calculate a maximum thermal modulus, which corresponds to the section of the part with the greatest thickness, and a minimum thermal modulus, which corresponds to the section of the part with the lowest thickness, of the part;
b) Obtain the cooling rate (ºC/s) for the maximum and minimum thermal moduli considering air cooling, said cooling rates being extracted from a cooling curve experimentally obtained from several samples having different thermal moduli;
c) Calculate the minimum cooling rate (CRₘᵢₙ) needed to avoid the pearlitic nose, as a function of different contents of Ni, Cu and Mo (wt.%) comprised in a chemical composition of the iron part, in which said contents of Ni, Cu and Mo vary as follows:
Ni: 3.0 - 5.0 % in wt,
Mo: 0.0 - 0.2 % in wt,
Cu: 0.0 - 1.0 % in wt
wherein the minimum cooling rate (CRₘᵢₙ) is calculated using the following formula:
d) Select one of said compositions with a minimum cooling rate (CRₘᵢₙ) lower than the cooling rate for the maximum thermal modulus;
e) Calculate the eutectoid temperature (T_{eutectoid}, ºC) as a function of the thermal modulus for the composition selected, for all the different thermal moduli of the part;
f) Calculate the shakeout temperature (Tₛₕₐₖₑₒᵤₜ, ºC) for each thermal modulus of the part;
g) Identify if the shakeout temperature Tₛₕₐₖₑₒᵤₜ for the minimum thermal modulus is over the eutectoid temperature (T_{eutectoid}) calculated in e) and if the shakeout temperature Tₛₕₐₖₑₒᵤₜ for the maximum thermal modulus is below the solidus temperature (T_{solidus}, ºC);
h) Select among the Tₛₕₐₖₑₒᵤₜ, the lowest temperature,
i) Calculate the isothermal transformation temperature T_{isothermal_transformation} for each thermal modulus of the part.
j) Identify if the isothermal transformation temperature T_{isothermal_transformation} for the minimum and maximum thermal moduli are between 450ºC and 170 ºC.
k) Select among the isothermal transformation temperatures Tᵢₛₒₜₕₑᵣₘₐₗ transformation, the one that better fits the targeted mechanical properties.

2. - The method of claim 1, wherein the step b) comprises the following steps:
b1) Obtain continuous cooling transformation (CCT) diagrams for several alloys with different contents of Ni, Cu and Mo.
b2) Consider the cooling curves obtained in step b1) as straight lines on the temperature range from 600ºC to 700 ºC and represent the slope of the lines in a cooling rate/thermal modulus diagram.
b3) Obtain a regression line for the slopes of step b2).

3. The method of claim 1, wherein in the step e) the eutectoid temperature (T_{eutectoid}) as a function of the thermal modulus is calculated using the formula:

4. The method of claim 1, wherein in the step f) the shakeout temperature (Tₛₕₐₖₑₒᵤₜ) for the different thermal moduli is calculated using the formula:

5. The method of claim 1, wherein step g) comprises identifying if Tₛₕₐₖₑₒᵤₜ for the minimum thermal modulus is over the eutectoid temperature + 50 ºC and if Tₛₕₐₖₑₒᵤₜ for the maximum thermal modulus is below the solidus temperature - 50ºC, wherein the upper limit for the section of the maximum thermal modulus to be shaken out is a temperature of 1050ºC.

6. The method of claim 1, wherein in the step i) the isothermal transformation temperature is calculated using the formula:

7. The method of claim 1, which further comprises the step of:
l) Calculate the ultimate tensile strength (UTS) of a given thermal modulus using the following formula:

8. The method of claim 1, which further comprises the step of:
m) Calculate the theoretical hardness (HB) of the parts using the following formula:

9. The method of claim 1, which further comprises the steps of:
ll) Calculate the optimum isothermal transformation temperature using the following formula:

10. The method of claim 1, which further comprises the steps of:
mm) Calculate the optimum isothermal transformation temperature using the following formula:

11. The method of claim 1, wherein the minimum thermal modulus of the part is greater than 0.4 and the maximum thermal modulus of the part is lower than 1.5.

## Patentansprüche

1. Verfahren zur Steuerung der ausferritischen Mikrostruktur im Gusszustand in einem Verfahren zum Erhalten von Eisenteilen mit Abschnitten unterschiedlicher Dicke, umfassend:
a) Berechnen eines maximalen Wärmemoduls, der dem Abschnitt des Teils mit der größten Dicke entspricht, und eines minimalen Wärmemoduls, der dem Abschnitt des Teils mit der geringsten Dicke des Teils entspricht;
b) Erhalten der Kühlrate (°C/s) für das maximale und minimale Wärmemodul unter Berücksichtigung der Luftkühlung, wobei die Kühlraten aus einer Kühlkurve extrahiert werden, die experimentell aus mehreren Proben mit unterschiedlichen Wärmemodulen gewonnen wurde;
c) Berechnen der minimalen Kühlrate (CRₘᵢₙ), die erforderlich ist, um die perlitische Nase zu vermeiden, als Funktion verschiedener Gehalte an Ni, Cu und Mo (Gew.-%), die in einer chemischen Zusammensetzung des Eisenteils enthalten sind, wobei die Gehalte an Ni, Cu und Mo wie folgt variieren:
Ni: 3,0 - 5,0 % im Gewicht,
Mo: 0,0 - 0,2 % im Gewicht,
Cu: 0,0 - 1,0 % im Gewicht,
wobei die minimale Kühlrate (CRₘᵢₙ) unter Verwendung der folgenden Formel berechnet wird: ${CR}_{min} \left(°C/s\right) = 2,35 - 0,33 ∗ Ni \left(Gew.-%\right) - 0.1 ∗ Cu \left(Gew.-%\right) - 4.0 ∗ Mo \left(Gew.-%\right)$
d) Wählen einer der Zusammensetzungen mit einer minimalen Kühlrate (CRmin), die niedriger ist als die Kühlrate für den maximalen Wärmemodul;
e) Berechnen der Eutektoidtemperatur (T_{eutektoid}, °C) in Abhängigkeit vom Wärmemodul für die gewählte Zusammensetzung für alle verschiedenen Wärmemodule des Bauteils;
f) Berechnen der Umstrukturierungstemperatur (Tₛₕₐₖₑₒᵤₜ, °C) für jeden Wärmemodul des Teils;
g) Identifizieren, ob die Umstrukturierungstemperatur Tₛₕₐₖₑₒᵤₜ für den minimalen Wärmemodul über der in e) berechneten Eutektoidtemperatur (T_{eutektoid}) liegt und ob die Umstrukturierungstemperatur Tₛₕₐₖₑₒᵤₜ für den maximalen Wärmemodul unter der Solidustemperatur (T_{solidus} °C) liegt;
h) Auswählen der niedrigsten Temperatur unter den Tₛₕₐₖₑₒᵤₜ;
i) Berechnen der isothermen Umwandlungstemperatur T_{isotherm_transformation} für jeden Wärmemodul des Teils;
j) Identifizieren, ob die isotherme Umwandlungstemperatur T_{isothermal_transformation} für die minimalen und maximalen Wärmemodule zwischen 450 °C und 170 °C liegt;
k) Auswählen unter den isothermen Umwandlungstemperaturen T_{isothermal_transformation} diejenige, die den angestrebten mechanischen Eigenschaften am besten entspricht.

2. Verfahren nach Anspruch 1, wobei der Schritt b) die folgenden Schritte umfasst:
b1) Erhalten von Diagrammen zur kontinuierlichen Abkühlungstransformation (CCT) für mehrere Legierungen mit unterschiedlichen Gehalten an Ni, Cu und Mo.
b2) Betrachten die in Schritt b1) erhaltenen Abkühlkurven als gerade Linien über dem Temperaturbereich von 600 °C bis 700 °C und repräsentieren der Steigung der Linien in einem Kühlraten-/Wärmemoduldiagramm.
b3) Erhalten einer Regressionslinie für die Steigungen von Schritt b2).

3. Verfahren nach Anspruch 1, wobei in Schritt e) die Eutektoidtemperatur (T_{eutektoid}) als Funktion des Wärmemoduls unter Verwendung der Formel berechnet wird: ${T}_{Eutektoid M} \left(°C\right) = - 41,93 ∗ {M}^{2} \left(cm2\right) + 115,03 ∗ M \left(cm\right) + 593,24$

4. Verfahren nach Anspruch 1, wobei in Schritt f) die Umstrukturierungstemperatur (Tₛₕₐₖₑₒᵤₜ) für die verschiedenen Wärmemodule unter Verwendung der Formel berechnet wird: ${T}_{shakeout M} \left(°C\right) = 568,40 ∗ M \left(cm\right) - 341,04 + {T}_{shakeout 0,6 cm} \left(°C\right)$

5. Verfahren nach Anspruch 1, wobei Schritt g) das Identifizieren umfasst, ob Tₛₕₐₖₑₒᵤₜ für den minimalen Wärmemodul über der Eutektoidtemperatur +50 °C liegt und ob Tₛₕₐₖₑₒᵤₜ für den maximalen Wärmemodul unter der Solidustemperatur -50 °C liegt, wobei die obere Grenze für den Abschnitt des maximalen umzustrukturierenden Wärmemoduls eine Temperatur von 1050 °C ist.

6. Verfahren nach Anspruch 1, wobei in Schritt i) die isotherme Umwandlungstemperatur unter Verwendung der Formel berechnet wird: ${T}_{isothermal transformation M} \left(°C\right) = 293,39 ∗ M \left(cm\right) + {T}_{isothermal transformation 0,6 cm} \left(°C\right) - 180$

7. Verfahren nach Anspruch 1, das ferner den Schritt umfasst:
l) Berechnen der Bruchzugfestigkeit (UTS) eines gegebenen Wärmemoduls unter Verwendung der folgenden Formel: $UTS \left(MPa\right) = - 1,2231 ∗ {T}_{isothermal transformation M} \left(°C\right) + 1308.2$

8. Verfahren nach Anspruch 1, das ferner den Schritt umfasst:
m) Berechnen der theoretischen Härte (HB) der Teile unter Verwendung der folgenden Formel: $HB = - 0,483 ∗ {T}_{isothermal transformation M} \left(°C\right) + 466,34$

9. Verfahren nach Anspruch 1, das ferner die Schritte umfasst:
ii) Berechnen der optimalen isothermen Umwandlungstemperatur unter Verwendung der folgenden Formel: ${T}_{isothermal transformation M} \left(°C\right) = - 0,8176 ∗ UTS \left(MPa\right) + 1069,58$

10. Verfahren nach Anspruch 1, das ferner den Schritt umfasst:
mm) Berechnen der optimalen isothermen Umwandlungstemperatur unter Verwendung der folgenden Formel: ${T}_{isohtermal transformation M} \left(°C\right) = 965,50 - 2.070 ∗ HB$

11. Verfahren nach Anspruch 1, wobei der minimale Wärmemodul des Teils größer als 0,4 und der maximale Wärmemodul des Teils kleiner als 1,5 ist.

## Revendications

1. Procédé de commande de la microstructure ausferritique brute de coulée dans un procédé pour obtenir des pièces en fer avec des sections de différentes épaisseurs, qui comprend :
a) le calcul d'un module thermique maximal, qui correspond à la section de la pièce ayant la plus grande épaisseur, et d'un module thermique minimal, qui correspond à la section de la pièce ayant la plus faible épaisseur, de la pièce ;
b) l'obtention de la vitesse de refroidissement (°C/s) pour les modules thermiques maximal et minimal compte tenu du refroidissement par l'air, lesdites vitesses de refroidissement étant extraites d'une courbe de refroidissement obtenue de façon expérimentale à partir de plusieurs échantillons ayant différents modules thermiques ;
c) le calcul de la vitesse de refroidissement minimale (CRₘᵢₙ) nécessaire pour éviter le nez perlitique, en fonction de différentes teneurs en Ni, Cu et Mo (% en poids) comprises dans une composition chimique de la pièce en fer,
dans lequel lesdites teneurs en Ni, Cu et Mo varient comme suit :
Ni : 3,0 à 5,0 % en poids,
Mo : 0,0 à 0,2 % en poids,
Cu : 0,0 à 1,0 % en poids
dans lequel la vitesse de refroidissement minimale (CRₘᵢₙ) est calculée en utilisant la formule suivante : ${CR}_{min} \left(°C/s\right) = 2,35 - 0,33 * Ni \left(% en poids\right) - 0,1 * Cu \left(% en poids\right) - 4,0 * Mo \left(% en poids\right)$
d) la sélection d'une desdites compositions avec une vitesse de refroidissement minimale (CRₘᵢₙ) inférieure à la vitesse de refroidissement pour le module thermique maximal ;
e) le calcul de la température eutectoïde (T_{eutectoïde}, °C) en fonction du module thermique pour la composition sélectionnée, pour tous les modules thermiques différents de la pièce ;
f) le calcul de la température de décochage, démoulage, (T_{décochage}, °C) pour chaque module thermique de la pièce ;
g) déterminer si la température de décochage T_{décochage} pour le module thermique minimal est au-dessus de la température eutectoïde (T_{eutectoïde}) calculée en e) et si la température de décochage T_{décochage} pour le module thermique maximal est en-dessous de la température de solidus (T_{solidus}, °C) ;
h) la sélection, parmi les T_{décochage}, de la température la plus basse ;
i) le calcul de la température de transformation isotherme T_{transformation_isotherme} pour chaque module thermique de la pièce ;
j) déterminer si la température de transformation isotherme T_{transformation_isotherme} pour les modules thermiques minimal et maximal est comprise entre 450 °C et 170 °C ;
k) la sélection, parmi les températures de transformation isotherme T_{transformation_isotherme}, de celle qui correspond le mieux aux propriétés mécaniques ciblées.

2. Procédé selon la revendication 1, dans lequel l'étape b) comprend les étapes suivantes :
b1) obtention de diagrammes de transformation refroidissement continus (CCT) pour plusieurs alliages avec différentes teneurs en Ni, Cu et Mo.
b2) considérer les courbes de refroidissement obtenues dans l'étape b1) comme étant des lignes droites dans la plage de température de 600 °C à 700 °C et représenter la pente des droites dans un diagramme taux refroidissement/module thermique.
b3) obtention d'une droite de régression pour les pentes de l'étape b2).

3. Procédé selon la revendication 1, dans lequel, dans l'étape e), la température eutectoïde (T_{eutectoïde}) en fonction du module thermique est calculée en utilisant la formule : ${T}_{eutectoïdeM} \left(°C\right) = - 41,93 * {M}^{2} \left({cm}^{2}\right) + 115,03 * M \left(cm\right) + 593,24 .$

4. Procédé selon la revendication 1, dans lequel, dans l'étape f), la température de décochage (T_{décochage}) pour les différents modules thermiques est calculée en utilisant la formule : ${T}_{décochageM} \left(°C\right) = 568,40 * M \left(cm\right) - 341,04 + {T}_{décochage 0 6 cm} \left(°C\right) .$

5. Procédé selon la revendication 1, dans lequel l'étape g) comprend le fait de déterminer si T_{décochage} pour le module thermique minimal est au-dessus de la température eutectoïde + 50 °C et si T_{décochage} pour le module thermique maximal est en-dessous de la température de solidus - 50 °C, dans lequel la limite supérieure pour la section du module thermique maximal de décochage est une température de 1050 °C.

6. Procédé selon la revendication 1, dans lequel, dans l'étape i), la température de transformation isotherme est calculée en utilisant la formule : ${T}_{transformation _ isothermeM} \left(°C\right) = 293,39 * M \left(cm\right) + {T}_{transformation _ isotherme 0,6 cm} \left(°C\right) - 180 .$

7. Procédé selon la revendication 1, qui comprend en outre l'étape de :
l) calcul de la résistance ultime à la traction (UTS) d'un module thermique donné en utilisant la formule suivante : $UTS \left(MPa\right) = - 1,2231 * {T}_{transformation _ isothermeM} \left(°C\right) + 1308,2 .$

8. Procédé selon la revendication 1, qui comprend en outre l'étape de :
m) calcul de la dureté théorique (HB) des pièces en utilisant la formule suivante : $HB = - 0,483 * {T}_{transformation _ isothermeM} \left(°C\right) + 466,34 .$

9. Procédé selon la revendication 1, qui comprend en outre les étapes de :
ll) calcul de la température de transformation isotherme optimale en utilisant la formule suivante : ${T}_{transformation _ isothermeM} \left(°C\right) = - 0,8176 * UTS \left(MPa\right) + 1069,58 .$

10. Procédé selon la revendication 1, qui comprend en outre les étapes de :
mm) calcul de la température de transformation isotherme optimale en utilisant la formule suivante : ${T}_{transformation _ isothermeM} \left(°C\right) = 965,50 - 2,070 * HB .$

11. Procédé selon la revendication 1, dans lequel le module thermique minimal de la pièce est supérieur à 0,4 et le module thermique maximal de la pièce est inférieur à 1,5.
